# EUROPEAN PATENT APPLICATION

(11) **EP 1 707 657 A1**
(43) Date of publication of application: **04.10.2006**
(21) Application number: 05075753.3
(22) Date of filing: 31.03.2005
(51) Int. Cl.: D04H 1/70, D04H 1/42, D04H 1/54

(54) **Process for producing elastic and/or water degradable webs from composite filaments**

(71) Applicant: M & J Fibretech A/S, 8700 Horsens (DK)
(72) Inventor: Andersen, Jens Ole Bröchner, 8660 Skanderborg (DK)
(74) Representative: Holme Patent A/S

(57) **Abstract**

A process of manufacturing a non-woven web from virtually endless composite filaments (1). The filaments used in said process are arranged in a sheath-core arrangement in which the sheath component (3) comprise a thermoplastic polymer and the core (2, 2') is selected from the group of an elastomer, a water-soluble polymer and/or a biodegradable polymer. The process according to the invention provides a simple and inexpensive process for manufacturing water soluble and/or elastic non-woven webs of any width, using virtually endless filaments.

## Description

The present invention relates to a process for producing elastic and/or water-soluble and/or water degradable webs from composite filaments. The invention further relates to the webs obtainable by said process and the filaments used in said process.

Non-woven webs are used in the manufacture of a variety of products such as bandaging materials, garments, diapers, incontinence products, support clothing, and personal hygiene products. These articles are normally designed to absorb and contain bodily fluids and at the same time provide a physical barrier to such fluids. In order to allow more freedom of body movement the articles can advantageously be elastic.

Products of the kind named above are conventionally disposed as normal household waste, and thereafter either placed in landfills or combusted. Either way, the waste constitute a potential environmental hazard, and the demand to reduce the amount of everyday waste is growing.

Manufactures of the article are presently trying to solve these problems by making the articles flushable.

It should in this respect be noted, that there are no common definition of the term flushable. The term is used at random when a product fits down the toilet, not taking into consideration what happens to the product after it enters the sewage system.

While there are several types of flushable articles on the market for toilet cleaning, kids care and personal hygiene, these articles are not fully degradable and are therefore a threat to municipal septic and sewer systems nationally.

Non-woven webs are conventionally produced by a variety of methods, but only the well known spunbond" process is capable of utilising long fibre filaments.

In the "spunbond" process, filaments of one or more molten polymers are extruded from a large number of orifices formed in a spinnerette plate. The filaments are immediately thereafter stretched or drawn, and are then randomly deposited upon a collection surface to form a non-woven web. The stretching or attenuation can be mechanically through the use of draw rolls, or, as is more widely practiced, pneumatically by passing the filaments through a pneumatic attenuator.

Manufacturers of spunbonded non-woven fabrics have long sought to improve the manufacturing process to achieve higher productivity and better quality and uniformity of the spunbonded non-woven fabric. Maintaining the quality and uniformity of the fabric becomes a particular concern at higher production speeds and when producing fabrics of low basis weight.

While spunbond materials with desirable combinations of physical properties, especially combinations of softness, strength and durability, have been produced, significant problems have been encountered.

One main problem is attributed to the fact that the width of the non-woven webs manufactured with the spundbonding process is limited by the width of the spinnerette plate, as this plate has to be arranged across the whole width of the production line. Manufacturing broad non-woven webs by such process therefore requires larges unremunerative production plants.

It has therefore in practice, been necessary to reach a compromise where a plant is operated with relatively small width of web, resulting in that the capacity of the plant is far from being fully utilized.

Another problem with the spundbond process relates to the manufacture of e.g. elastic non-woven webs. Elastic fibres have a characteristic "sticky" nature, as these fibres normally comprise elastomers. Spunbonding, which employ air drawing, can be particularly effected. For example, turbulence in the air can bring filaments into contact and these "sticky" filaments can then adhere to one another. This stickiness proves to be especially troublesome during winding of the webs into rolls. The layers of web adhere to one another, a phenomenon known as "blocking".

While it can be possible to decrease the effect of the stickiness of the elastic filaments, this involves further process steps, and therfore introduce a significant complication into the process for producing an elastic non-woven web. Such complications can result in a significant addition to the cost of the resulting fabric.

Separately, attempts have been made to influence the properties of fabrics by modifying the content of the fibers, e.g. by combining polymers in bi-and multicomponent fibres.

One example of a bi-component elastic fibre is known from US Patent No. 5,352,518, and use of such filaments in the spundbonding process reduces some of the drawbacks, but the limited production width of the web using the spundbonding process still add additional costs to the final product.

Furthermore, these filaments have faced problems such as breakage or elastic failure of the strand during extrusion and/or drawing. Broken strands can clog the flow of filaments and/or mesh with other filaments, resulting in the formation of a mat of tangled filaments in the web.

While the art has sought to address the foregoing problems, it is clear that the results have, at best, been mixed.

It is therefore a first aspect according to the present invention, to provide a simple and inexpensive process for manufacturing non-woven webs of any width, using virtually endless filaments.

It is a second aspect according to the present invention to provide a water soluble or elastic non-woven web produced by the process according to the invention at low cost.

It is a third aspect according to the present invention to provide a novel elastic filament.

It is a forth aspect according to the present invention to provide a novel water-soluble and/or biodegradable filament.

It is a fifth aspect of the present invention to provide a non-woven web comprising the filaments according to the invention, which gives an excellent feeling to wearers.

It is a sixth aspect of the present invention to provide a non-woven web, which is fully degradable in water.

The new and unique way in which the present invention fulfills the above mentioned aspects is that the process comprises the following steps, defibrating a fibre material comprising the filaments, transporting the defibrated fibre material to at least one forming head and forming a non-woven web on an endless forming wire. The filaments are arranged in a sheath-core arrangement in which the sheath component comprise a thermoplastic polymer and the core is selected from the group comprising an elastomer, a water-soluble polymer and a biodegradable polymer.

During the initial cutting step the virtually endless filaments will be divided into smaller segments and/or fibres, enabling these fibres to be used in e.g. a conventional airlaying process. Thereby is not only obtained the advantage that elastic webs and/or water soluble webs can be formed in a more simple and more economical process than hitherto known, but also, that virtually endless filaments can be used in these process.

It should in this respect be mentioned, that conventional airlaying process in some instances include a defibration step, however this step relates to unwind and open fluff pulp not to defibration long filaments. The difference can especially be found as no rolled up fiber lumps, collectively known as nits, are formed during the defibration of the filaments, which normally possess an extreme problem during the conventional defibration of fluff pulp.

Furthermore, the process according to the invention further provides the advantages, that the width of the web can be much broader, as the spinneret used to manufacture the filaments have no effect on the dimensions of the final web, as in the conventional spunbonding process. The spinneret used to prepare the filaments before they are being defibriated, can therefore have a lesser dimension, ensuring that the spinneret occupies lesser space in the plant.

Alternatively, the spinneret can be separate from the production plant, as the filaments do not have to be produced simultaneously with the web. Furthermore, filaments of different weights and/or physical and/or chemical properties can in an advantageously embodiment be defibriated in the process according to the invention either simultaneously or at different stages of the process. Thereby, the process according to the invention is not only very flexible, as webs will several layers with different properties or weights easily can be produced with the process according to the invention, the process according to the invention is also a more simple and economical process than hitherto known.

As an example can be mentioned, that the filaments e.g. can be produced with weights from 0.3 dtex to 25 dtex, and that webs manufactured with these filaments provide webs with characteristics and qualities not previously known from corresponding webs.

The process according to the invention can further include opening and feeding short cut staple fibre and dose superabsorbents or other powders to one or more forming heads. These materials can be suspended in air within a forming system and deposited on a moving forming screen or rotating perforated cylinder.

As the sheath of the filaments comprises a thermoplastic polymer this polymer will be activated during a subsequent thermal bonding step. During said step, the web can e.g. pass through a through-air oven, which activates the synthetic fibres, binding the web components together. After activation the product is calendered to the correct thickness and cooled before it is winded into jumbo rolls. Thermally bonding a web involves applying heat and pressure via a calendar to consolidate the web. Therefore, it is adventurously that the sheath component has a lower melting temperature than the core.

To have an economic process the sheath component should preferably be a thermoplastic polymer having a very low melting point, such as a polyamide, polyester or polyolefin.

During the thermal bonding step the sheath polymer will melt and be concentrated in the junctions between the fibres, thereby, at least partly, uncovering the core. The properties of the core can then be utilised optimally, while at the same time obtaining a strong web.

The person skilled in the art would understand, that the process according to the present inventions could utilise either bi- or mulicomponent filaments. Thus, the core does not have to be a single unit and can be made up of several independent elements, which can be composed of the same or different polymer/elastomer. Furthermore, the different core elements can be either uniformly or randomly distributed in the sheath component. Simmilar, the sheath component can be composed of several different layers, or can be a mixture of different thermoplastic polymers.

The nature of the final web are determined by the nature of the filaments, thus when the core is an elastomer the final web will be an elastic web and when the core is a water-soluble polymer and/or a biodegradable polymer the web will e.g. be capable of dissolving in water.

The inventors have surprisingly found that when the sheath component is present in an amount of at least 60 weight%, based on the weight of the total filament, the filaments have the advantage, compared to conventional composite filaments, that they will not break during their preparation, i.e. during the the extrusion and/or drawings step of the manufacture. These filaments will therefore never clog the flow of filaments and/or mesh with other filaments, and the problem with tangled filaments is therefore eliminated. Contents of at least 65, or at least 70-weight% are even more preferred according to the invention.

When filaments having the above-mentioned composition the process furthermore provides a non-woven web with a desirable combinations of physical properties, especially combinations of softness, strength and durability.

According to one embodiment of the present invention the core is an elastomer.

By elastomer is meant an amorphous, cross-linked high polymer which will stretch rapidly under tension, reaching high elongations (500 to 1000%) with low damping. It has high tensile strength and high modulus when fully stretched. On the release of stress, it will retract rapidly, exhibiting the phenomenon of snap or rebound, to recover its original dimensions. Elastomers are unlike thermoplastics in that they can be repeatedly softened and hardened by heating and cooling without substantial change in properties.

When the core is an relatively cheep elastomer, e.g. polyolefin - such as polypropylen - or a styrenic elastomers the resultant webs can advantageously be used as disposable articles such as diapers, training pants or incontinence garments. The elastomer will provide the articles with a close, comfortable fit about the wearer and contain body exudates while maintaining skin health.

In other more durable products, such as waist elastics, leg elastics, elasticised liners, and elasticised outer covers i.e. elastic products with multi-use applications, the elastic condensation polymers such as polyurethane and copolyester, can advantageously be applied. These elastic components are employed to help produce and maintain the fit of the articles about the body contours of the wearer thereby leading to improved containment and comfort.

The elastic web of an embodiment of the present invention can be combined with one or more webs to provide a soft texture that may be more useful or appealing in some applications. Such webs can be fibrous in nature, examples being nonwoven and woven materials. One embodiment of the invention includes a composite material that comprises the elastic web described previously and an additional web. The composite material may be prepared by laminating the webs together, coextrusion, or any other suitable method for making the composite material.

Embodiments of the present invention provide elastic materials that contain apertures and are breathable when stretched, and in particular, breathable when stretched by a tensile force acting in the direction of the force that the material would experience in end use conditions (e.g., in a diaper side tab that would normally experience the hoop stress of the diaper waist band when gripping the wearer's waist). Another example of stress in the direction of the force that the material would experience in end use conditions includes the stress that would be experienced by a bandage that is wrapped in around a body part, or that is stretched and then adhered.

In another embodiment according to the present invention the core is a water-soluble polymer and/or a biodegradable polymer, ensuring that the web will disintegrate when it comes into contact with water. The core can be of any material that is adequately soluble and that will give appropriate properties to the final product. Preferably it has low oxygen permeability when dry. It can be, for instance, a polyethylen oxide (PEO) or a polyvinyl alcohol (PVOH).

PVOH are generally made by hydrolysis from polyvinyl acetate and the degree of hydrolysis affects solubility. Thus the degree of hydrolysis can be selected depending on the application of the final product.

Fully hydrolysed PVOH's (e.g., hydrolysed to an extent of at least about 98%) tend to be readily soluble only in warm or hot water. Thus if the final product are to be used as e.g. water soluble toilet paper it is preferred to use grades of polyvinyl alcohol which are not quite so fully hydrolysed, as the less hydrolysed grades tend to dissolve more readily in cold water and water with room temperature, e.g. 10 °C til 25°C. Therefore partially hydrolysed PVOH is preferably used, preferably having a degree of hydrolysis from polyvinyl acetate of 70 to 95%, most preferably 73 to 93%, when the product are to be applied in normal daily necessities.

PVOH used alone as a base polymer for the formation of a water-soluble web in the conventional techniques, suffers from several disadvantages. Due to PVOH's high melting point and poor thermal stability, it is very difficult to thermally process. An extruder, rather than merely a melt tank, is required to process the PVOH into a web. Additionally, once the web is formed, it has poor heat seal properties such that it would need to be heat sealed at temperatures that adversely affect the integrity of the substrate. The problems are solved by the present inventions, as the PVOH is sheathed with the thermoplastic polymer, ensuring that the PVOH easily can be processed into a thermally stabilised web.

The products comprising the water-soluble and/or degradable polymer produced according the present invention has a modified rate of water solubility i.e. they can both withstand to be exposed to the extremely varied strength requirements in the wet and dry states and at the same time dissolve in water after a specific time. The water-soluble core will namely be in direct contact with the water, as the thermal sheath polymer has melted during the thermal bonding step and concentrate in the junctions between the fibres, whereby the core is at least partly uncovered. The features of the core component can then be utilised optimally while at the same time obtaining a strong web.

For ensuring, that the webs according to the invention retain their strength at least for a specific period of time when exposed to aqueous liquids or moisture-containing food, the invention can adventurously comprise means for delaying the disintegrating when the article comes into contact with water. This can for instance be relevant in the case of household paper (kitchen towels). On the other hand, toilet paper must dissolve in water, some time after use, in order to prevent the sewage systems from clogging up. At the same time, wet toilet paper must not immediately loose its strength properties during use for apparent reasons.

Correspondingly, the prior art makes a distinction between dry strength and wet strength properties, the latter being divided in further categories such as initial wet strength, temporary wet strength and permanent wet strength depending on the point of time of measuring the wet strength after re-wetting a dry tissue paper.

In one embodiment the means for delaying the disintegration in water is a thin surface-coating, which is applied to the final article via conventional techniques. This ensures that the article is both capable of keeping the strength properties during use and at the same time that the article is capable of disintegrating in water. An example of such surface is a latex coating, but other coatings providing the same or similar properties can equally well be used. Coatings of this type are well known to the person skilled in the art.

As an alternative to a surface coating the product could e.g. be premoistened with a solution and/or wet-strength additives, which is not capable of dissolving the core or sheath-polymer.

If the web comprises PVOH, the web can advantageously be premoistened with a solution with a low salt concentration, as the salt will stabilise the bindings in the web. When the web is placed in contact with water having a lower salt concentration, the salt will be washed out, and the article will disintegrate.

Alternatively the article can be stabilised with calcium ions, which also stabilise the bindings in the web. When the article is immersed in water with less calcium or an excess of sodium ions, the solubility of the article increases.

If the polymer is PEO and/or PVOH said agent could preferably be saline with a relatively low salt concentration, of e.g. 1 M NaCl.

In preparing the premoistened article according to the invention, any of various suitable methods may be used. For example, the web may be saturated with the solution and then encapsulated or otherwise sealed in an airtight liquid impermeable package.

The premoistened article of the invention is ideally suited to be carried by a person in a packet or purse and, because it is premoistened, it is available immediately for use for wiping in a one-step cleaning operation.

In one embodiment of the invention a liquid disinfectant and/ or deodoriser is added to the premoistened solution, whereby the article functions to effectively cleanse, disinfect and deodorize.

The filaments according to the invention can preferable by used to produce articles designed to e.g. absorb and contain bodily fluids and/or provide a physical barrier to such fluids e.g. diapers, personal hygiene products or sanitary napkins.

The non-woven webs according to the invention can further be used in the manufacture of bandaging materials, garments, and support clothing.

The invention will be explained in greater detail below where further advantageous properties and example embodiments are described with reference to the examples and drawing:

### Figures

Fig. 1A-B, schematically illustrates the structure of two different embodiments of the filament according to the invention,
Fig. 2 is an electron-microscopy picture of an elastic web according to the invention.
Fig. 3 is an electron-microscopy picture of a biodegradable web according to the invention.

Below, the invention is described on the assumption that the core and sheath component is circular, however the invention is not limited to this specific structure. Thus, the core and/or sheath component can have other structures, such as hexagonal or triangular, with similar, or in some cases better, technical advantages, depending on the resultant web.

Fig. 1A is a schematic view of a filament 1 according to the invention. The filament 1 is designed with a core 2 and a circumferential sheath component 3.

The sheath component 3 comprises a thermoplastic polymer and the core 2 can be an elastomer, a water-soluble polymer and/or a biodegradable polymer, depending on the desired features of the final product.

In fig. 1B is the core 2 divided into a number of core-elements 4, 5 uniformly distributed in the center of the sheath component 3. In the present case is part of the elements an elastomer 4, and the rest of the elements an water degradable polymer 5. The sheath component 3 is spread between the elements 4,5. When the sheath polymer melt during the thermal bonding step the different core-elements 4,5 will be exposed, and the resultant web will be both elastic and water-degradable.

Fig. 2 and fig. 3 are respectively electron-microscopy pictures of elastic and a biodegradable webs according to the invention.

As illustrated by the arrows in said figures, it is evident, that the sheath component which has been melted during the thermal bonding step, has flow towards the junctions between the fibres where it has concentrated, thereby uncovering the core 2, at least partly. The properties of the core will then be able to be utilised optimally, while at the same time obtaining a strong web.

### Examples:

### Example 1: Manufacture of the filament

Fibre material having the general configuration of a sheath-core arrangement is prepared form molten polymers of the respective sheet-core polymers.

The molten polymers are formed in a batch process were they are forced through an extrusion head forming a spaghetti type product, which is cooled down and passed through a chip cutter where it is cut into so called chips.

In order to manufacture the bicomponent fibre material the different chips are fed onto two separate extruders, one for the sheet component and one for the core. Electrically heated zones around the cylinder in the extruder and high pressures caused by the action of the screw melt the chips and a fairly thick liquid results. The heating system keeps it in a molten state while it is fed at a controlled rate via spin or metering pumps into spin packs.

The molten polymers are forced through the spinnerette holes in the spin packs at a defined speed. To obtain the correct fibre thickness a constant pulling force is exerted by a roller arrangement, which draw the fibres down the spinning shafts.

The fibres formed by the spinnerette are still liquid and can adventurously be rapidly cooled down in order to solidify. For these purposes quench air is blown through the fibre bundle.

### Example 2: Air laying of the web.

The resulting filaments are fiberized in a defibration unit, and the resulting fibres are thereafter supplied to a forming head in the air laying plant by a fibre transport fan. The plant can be a multiple forming head systems. When each head is fed with its own unique blend of raw materials, it is possible to produce multilayer products, where each layer is engineered for a specific function in the product, for instance acquisition-distribution layer, absorption layer, barrier layer etc.

### Example 3: Elastic and/or water soluble non-woven webs

A bicomponent polyethylen fibre material (PEO-1), comprising 65-weight% polyolefin as a sheath component and 35-weight% polyethylen oxide as the core polymer was prepared as described in example 1.

A bicomponent polypropylen fibre material (PP-1), comprising 65-weight% polyolefin as a sheath component and 35-weight% polypropylen as the core polymer was prepared as described in example 1.

PEO-1 and PP-1 was used to produced a number of different webs, either alone, in combination or in blends with other material and/fibres, such as SAP, cellulose fibres.

All webs are manufactures according to the process described in example 1 and 2, resulting in webs with the following characteristics:

### Web 1

Wipes comprising between 15 and 25 weight% PEO-1, 0 to 15 weight% liquid binder and 60 to 85 weight% cellulose fibre were prepared. These wipes all showed a significant low wet strength and were completely disintegrated in tap water after only few minutes. These webs can therefore be considered completely flushable.

### Web 2

Wipes prepared from a homogenous web comprising 15 to 50 weight% PEO-1 and 50 to 85 weight% cellulose fibre. These wipes were not only soft but were also capable of being disintegrated in tap water.

### Web 3

However, a homogenous web with 100 weight% PEO-1, was not only disintegrated in water after few minutes.

### Web 4

Homogenous web with 50 weight% PEO-1 and 50 weight% elastic PP-1. This web was both elastic and capable of disintegrating in water.

### Web 5

Web comprising 35 to 65 weight% cellulose fibre, 35 to 65 weight% absorbent layer (SAP) and 3 to 15 weight% PEO-1. Also when the web comprised SAP was the web capable of being disintegrated in water.

### Web 7

- Top layer: 100 weight% synthetic PEO-1
- Middle 35 to: layer 65 weight% cellulose fibre , 35 to 65 to weight% absorbent layer and 3 to 15 weight% PEO-1.
- Bottom layer: 100 weight% very fine dtex PEO-1.

This web has a low wet strength ensuring that it was completely disintegrated in tap water after very few minutes.

### Web 8

- Top layer: 100 weight% synthetic PEO-1
- Middle layer: 35 to 65 weight% cellulose fibre, 35 to 65 weight% absorbent layer and 3 to 15 weight% PEO-1
- Bottom layer: 50 weight% very fine dtex PEO-1 and 50 weight% PP-1.

This web showed a low wet strength and were completely disintegrated in tap water after only very few minutes. The web further exhibited excellent elastic properties.

While particular embodiments of the present invention have been illustrated and described, it would be obvious to those skilled in the art that various other changes and modifications can be made without departing from the scope of the invention. It is therefore intended to cover in the appended claims all such changes and modifications that are within the scope of this invention.

## Claims

1. A process of manufacturing a non-woven web from a fibre material comprising composite filaments, said process comprises the following steps,
- defibrating the fibre material, ,(opening/dosing)
- transporting the defibrated fibre material to a forming head, **characterized in, that** the filaments is arranged in a sheath-core arrangement in which the sheath component comprise a thermoplastic polymer and the core is selected from the group of an elastomer, a water soluble polymer and/or a biodegradable polymer.

2. The process according to claim 1, **characterized in, that** the sheath component has a lower melting temperature than the core.

3. The process according to claim 1 or 2, **characterized in, that** the thermoplastic polymer is a polyamide, polyester or polyolefin.

4. The process according to claim 1, 2 or 3, **characterized in, that** water soluble polymer and/or a biodegradable polymer is a polyethylene oxide or a polyvinyl alcohol.

5. The process according to claim 1, 2 or 3, **characterized in, that** the elastomer is selected from the group comprinsing polypropylen, styrenic elastomer, polyurethane and copolyester.

6. The process according to any of the claims 1 - 5, **characterised in, that** the process further comprises a heating step.

7. A elastic filament as defined in claim 4, wherein the sheath component constitute from 60 to 70 weight% of the total filament and the core constitute from 40 to 30 weight% of the total filament.

8. A water-soluble and/or a biodegradable filament as defined in claim 4.

9. A non-woven web obtainable by the process according to any of the claims 1 - 6.

10. The non-woven web according to claim 9, premoistened with a solution and/or wet-strength additive.

11. Use of a non-woven web according to claim 9, in the manufacture of bandaging materials, garments, diapers, incontinence products, support clothing, and personal hygiene products.

12. Use of a non-woven web according to claim 9 or 10, in the manufacture of flushable article, such as diapers, personal hygiene products and cleaning pads.
